

## UNITED STATES PATENT OFFICE

2,569,477

## MAGNESIUM ALLOY

Thomas E. Leontis, Midland, Mich., assignor to  
 The Dow Chemical Company, Midland, Mich.,  
 a corporation of Delaware

No Drawing. Application October 3, 1949,  
 Serial No. 119,396

2 Claims. (Cl. 75—168)

1

The invention relates to an improved magnesium-base alloy exhibiting high creep resistance and tensile strength at elevated temperatures.

In an application for Letters Patent, Serial No. 119,395, filed concurrently herewith by me, now abandoned, there is set forth an improved magnesium-base alloy exhibiting high creep resistance and tensile strength at elevated temperatures which is based upon alloying neodymium and praseodymium with magnesium. Limited amounts of lanthanum normally associated with neodymium and praseodymium also may be present, although superior alloys are obtained without the lanthanum addition.

In further researches with the foregoing alloys, I have discovered that still greater improvement in creep resistance and elevated temperature tensile properties results when cerium is also alloyed with the magnesium along with the neodymium and praseodymium.

Accordingly, the alloy of the present invention consists of a base of magnesium with which is alloyed the three elements of the ceria earth group: cerium, neodymium, and praseodymium, their total amount being between about 1 and 10 per cent by weight of the alloy, the balance being magnesium and incidental impurities, if any. It has been found that the usual small amounts of other ceria metals normally associated with above-specified ceria metals may be present in limited amount in the alloy without significant detrimental effects. Except for lanthanum, which may amount to as much as 10 per cent of the ceria earth metal content of the alloy, the other minor ceria earth metal impurities are generally less than about 3 per cent of the specified ceria earth metal content of the alloy. These minor ceria earth metals include Sm, Tb, Y. Insofar as known, these minor practically unavoidable alloying constituents have no measurable effect on the tensile properties of creep resistance of the alloy.

One source of the metals neodymium and praseodymium for use in the alloy is commercial didymium which consists largely of these metals together with inconsequential amounts of some other ceria earth metals including sarmarium, terbium, yttrium and lanthanum which may be present in amount up to about 10 per cent of the ceria earth metal content of the didymium. The following is an example of a commercial didymium: Ce 0.8%, Nd 72.3%, Pr 7.9%, La 8.8% (by difference from the total ceria group rare earth metals content of 89.9%), Fe 7.05%, Si

0.56%, Cr 0.75%; other impurities 2.8% including small amounts of sarmarium, terbium, yttrium (by difference from 100%). The other ceria earth metal for use in the alloy, viz., cerium, normally contains small amounts of other ceria earth metals including neodymium, praseodymium and lanthanum in amount up to about 5 per cent of the weight of the cerium. The following is an analysis of a commercial cerium: Ce 92.2%, Nd 0.9%, Pr 0.3%, La 1.4% (by difference from the total rare earth metals content of 94.8%); Fe 2.37%, Si 0.02%, Cr 0.5%, other impurities 1.4% (by difference from 100%).

In preparing the alloy, the magnesium is preferably first melted and then the specified ceria earth metals are added. The melting of the magnesium is most suitably accomplished in an open top crucible using a thickening magnesium foundry flux for protection from the atmosphere. The usual thickening magnesium foundry flux may be used such as one composed of 20% KCl, 50% MgCl<sub>2</sub>, 15% CaF<sub>2</sub> and 15% MgO in amount between about 1 and 3 per cent of the weight of the melt, although other amounts may be used. The flux has the property of being fluid at the commencement of melting and becoming crust-like after prolonged heating so that a crust-like cover of dried flux forms over the melt after a time. Before the crust forms, the specified ceria earth metals are introduced into the molten magnesium, preferably by holding them in a ladle and moving the ladle about in the melt so as to wash out the rare earth metals from the ladle and disperse them through the melt. After alloying the specified rare earth metals with the melt, it is desirable to cast the alloy promptly to avoid loss of the added metal to the flux which, if it contains magnesium chloride, is slowly decomposed by these rare earth metals.

In the event that the alloy once made is to be remelted, a process in which the flux is ordinarily in contact with the metal for a relatively long time compared to the alloying time, it is desirable, if not necessary, to employ a saline flux, free from MgCl<sub>2</sub>, which remains fluid while molten, such as composed of 57% KCl, 28% CaCl<sub>2</sub>, 12.5% BaCl<sub>2</sub>, and 2.5% of CaF<sub>2</sub> in place of the crust-forming or thickening type of flux.

The following analysis is of an alloy made in accordance with the invention using the commercial didymium and cerium noted above: Ce 0.91%, Nd 0.54%, Pr 0.12%, La 0.12%, total rare earth 1.69%, balance magnesium of 99.7% purity.

The tensile properties are set forth, for the temperatures indicated, in Table I.

Table I

| Tempera-ture,<br>°F. | Per Cent<br>Elonga-tion in 2<br>Inches | Load in 1,000's, p. s. i. |      |
|----------------------|----------------------------------------|---------------------------|------|
|                      |                                        | TYS                       | TS   |
| Room                 | 3.7                                    | 13.5                      | 27.1 |
| 400                  | 12.5                                   | 13.4                      | 20.1 |
| 600                  | 35.5                                   | 10.0                      | 12.5 |

TYS=Tensile yield strength, the stress at which the stress strain curve deviates 0.2% from the modulus line.

TS=Tensile strength, the stress at which the ratio of stress to strain is a maximum.

The creep limits for 100 hours load application for the same alloy composition are set forth in Table II.

Table II

| Tempera-ture,<br>°F. | Load in 1,000's p. s. i. |                         |                         |
|----------------------|--------------------------|-------------------------|-------------------------|
|                      | 0.1% Creep<br>Extension  | 0.2% Total<br>Extension | 0.5% Total<br>Extension |
| 400                  | 0.8                      | 9.8                     | 11.2                    |
| 500                  | 5.2                      | 5.2                     | 6.0                     |
| 600                  | 2.1                      | 2.5                     | 2.7                     |

Although the cerium and didymium used in preparing the foregoing example of the alloy contains small amounts of lanthanum it is to be understood that the alloy of the invention can be compounded of lanthanum-free cerium and didymium with the advantage that still better high temperature properties are exhibited.

In general, the magnesium-base alloy of the invention may contain cerium and both praseodymium and neodymium in a range of proportions such that the cerium is from 25 to 75 per cent of the total of the rare earth metal content

of cerium, neodymium and praseodymium. A preferred proportion of cerium to the other two rare earth metals is an amount equal to the sum of the amounts of the other two.

It will be noted that the usual commercial forms of cerium and didymium contain minor amounts of other metals as impurities, such as iron, silicon and chromium. These impurities do not cause any harm because they are either insoluble in the magnesium and are, therefore, precipitated and settle out of the melt during alloying, or are present in such small amount as to produce no significant effects in the final alloy.

I claim:

1. A magnesium-base alloy containing the rare earth metals cerium, neodymium and praseodymium, the balance being magnesium, the amount of said rare earth metals totaling between about 1 and 10 per cent of the weight of the alloy, the proportion of cerium being 25 to 75 per cent of the total amount of rare earth metal, and the amount of neodymium being at least four times that of the praseodymium.

2. A magnesium-base alloy containing about 0.9 per cent of cerium, 0.54 per cent of neodymium, 0.12 per cent of praseodymium, and 0.12 per cent of lanthanum, the balance being magnesium.

THOMAS E. LEONTIS.

#### REFERENCES CITED

The following references are of record in the file of this patent:

#### UNITED STATES PATENTS

| Number    | Name                  | Date          |
|-----------|-----------------------|---------------|
| 2,121,292 | Haughton et al. ....  | June 21, 1938 |
| 2,221,319 | Altwicker et al. .... | Nov. 12, 1940 |
| 2,464,918 | Ball et al. ....      | Mar. 22, 1949 |

#### FOREIGN PATENTS

| Number  | Country            | Date         |
|---------|--------------------|--------------|
| 342,586 | Great Britain .... | Feb. 5, 1931 |